

## UNITED STATES PATENT OFFICE

LESLIE WALTER OLIVER AND WILLIAM GEORGE CLARE, OF LONDON, ENGLAND, AS  
SIGNORS TO COLOUR PHOTOGRAPHS (BRITISH AND FOREIGN) LIMITED, OF LONDON,  
ENGLAND, A BRITISH COMPANY

## PRINTING PROCESS EMPLOYED IN COLOR PHOTOGRAPHY

No Drawing. Application filed June 2, 1931, Serial No. 541,686, and in Great Britain June 23, 1930.

This invention comprises improvements in or relating to printing processes employed in color photography.

The invention relates to a process of the 5 type in which relief images obtained by differential hardening, by light or chemical action, are formed upon colloid layers carried on suitable supports.

A well known example of the above type 10 of process—and one with which the present invention is particularly concerned—is the so-called "carbon" or "carbro" process in which a picture in natural colors is obtained by printing from negatives taken through 15 colored filters on to carbon tissues dyed in the complementary colors. Usually in carrying out such a process the following procedure is adopted. The tissues, which consist essentially of a paper base coated with 20 a mixture of soluble gelatine and the appropriate coloring matter, are rendered sensitive to light by treatment with alkali dichromate solutions. After exposure, the tissues are soaked in water, squeegeed into contact with celluloid or other impervious supports and later immersed in warm water, when the paper backing and unexposed gelatine leaves the support and a colored image in hardened gelatine is left. The three images (which in a three-color process are colored respectively magenta, yellow and blue-green) may now be dried on their celluloid 25 supports and mounted in register. It is more usual however to transfer each developed image in turn from the celluloid support to a final paper base. This transference is rendered possible by coating the celluloid with a thin layer of wax before mounting the carbon tissue thereon for development. Unless 30 the wax is suitably chosen and applied the pigmented image is liable to leave the celluloid support during development (frilling) and in those cases where such frilling does not occur it often proves difficult to effect 35 the final transfer of the image from the celluloid to the final support. In those cases where the transference is successful it is necessary to remove the wax from the surface of the transferred image before the other 40 images can be mounted thereon.

With a view to overcoming the practical disadvantages of the process described above it has been proposed to employ, in place of celluloid and as a combined development and final support, a sheet of regenerated cellulose (particularly that known under the registered name "Cellophane") or like material which is transparent, homogeneous, permeable to water and retentive of its mechanical strength and toughness when wet. According 55 to the above proposal there was no transference from one support to another after development, and the three-color pictures were thus made up of three superimposed 60 sheets of cellophane each bearing one of the 65 three-color components.

While the use of regenerated cellulose as a final support presents distinct advantages over celluloid, special means must be taken 70 in order that the resultant color picture may remain flat under changing atmospheric conditions. Moreover, if it is desired to adjust the proportions of the constituent colors in the finished print—for example, to reduce the amount of yellow whilst leaving the other colors untouched—the presence in the finished picture of three isolating layers of cellophane render this operation difficult and uncertain in accomplishment and accordingly 75 such color balancing must be performed before the three tissues are mounted together.

The present invention provides a printing process of the type described (i. e. in which relief images obtained by differential hardening are formed on colloid layers) which is characterized by combining the use, as a support for the image during development, of regenerated-cellulose (particularly that known under the registered trade-mark "Cellophane") or like material which is transparent, homogeneous, permeable to water, and retentive of its mechanical strength and toughness when wet, with the transference of the developed image from its regenerated-cellulose or like support to another base such 85 as paper.

Thus according to the invention the advantages of using cellophane or the like as a support during development are retained, 90 while the difficulties attendant upon the pres- 95

ence of the cellophane sheets as part of the final picture are obviated.

In one method, according to the invention, of effecting the transference of the image from the cellophane to the final support, the sheet of cellophane bearing the developed image is first soaked in water until fully swollen and is then mounted face downwards upon a piece of gelatine coated paper. A dilute solution of gelatine can conveniently be used as the mountant. The sandwich is now dried partially or completely and is then immersed in a dilute solution of a gelatine hardening or tanning agent, for example dilute solutions of potash alum, chrome alum, formalin or acrolein. After a few minutes immersion in such a solution, the cellophane can be readily separated from the paper support and the colored image will be found to be adhering firmly to the latter. Whilst the above procedure provides the simplest means for accomplishing this transfer, it has been found that soaking of the dried sandwich in water alone is sufficient to enable the cellophane to be separated from the image. In this case, however, it is necessary to dry the sandwich almost completely and to soak in water solution for some considerable time before attempting to strip off the cellophane.

In general, in carrying out the invention an adhesive is used in mounting, or treatment is applied to the mounted sandwich such that the adhesion of the colored image to the chosen final support is rendered greater than its adhesion to the sheet of regenerated cellulose whereon it was developed.

It is to be understood that in carrying out the process according to this invention the final support need not necessarily be of paper; other materials such as ivory, glass, canvas, silk or metal may be employed. Where a metal surface is used as the final support the transferred image may provide a suitable relief for an etching process such as photogravure. Transference to the curved metal surfaces commonly used in photogravure is not practicable from semi-stiff water-impermeable development supports such as celluloid and in consequence it has up till now been common practice to develop the carbon image directly on to the metal. With such practice the production of suitable reliefs is entirely dependent on the skill of the operatives. However by employing as development supports sheets of flexible water-permeable material such as cellophane it is possible to determine the suitability of the reliefs before transferring them to the cylinders.

We claim:

1. In a color-photographic printing process in which relief images obtained by differential hardening are formed on colloid layers, a method of transferring the developed image from a temporary support of regenerated cel-

lulose to a final base of another material which consists in soaking the image-bearing sheet in water until fully swollen, then mounting it face downwards upon the final support using a dilute solution of gelatine as a mountant, partially drying the sandwich, then immersing it in a dilute solution of a gelatine hardening agent, and finally stripping off the development support.

2. In a color-photographic printing process in which relief images obtained by differential hardening are formed on colloid layers, a method of transferring the developed image from a temporary support of regenerated cellulose to a final base of another material which consists in soaking the image-bearing sheet in water until fully swollen, then mounting it face downwards upon the final support using a dilute solution of gelatine as a mountant, completely drying the sandwich, soaking it in water and finally stripping off the development support.

3. In color photography a printing process which comprises developing, by differential hardening, a relief image on a colloid layer supported upon a sheet of regenerated cellulose, combined with transferring the developed image from its aforesaid regenerated cellulose support to another and final base by first soaking the image-bearing sheet in water until fully swollen, then mounting it face downwards upon the final base using an adhesive solution as a mountant, then drying the sandwich thus formed, and finally stripping off the development support.

4. In color photography a printing process which comprises developing, by differential hardening, a relief image on a colloid layer supported upon a sheet of regenerated cellulose, combined with transferring the developed image from its aforesaid regenerated cellulose support to another and final base of gelatine-coated paper by first soaking the image-bearing sheet in water until fully swollen, then mounting it face downwards upon the gelatine-coated surface of the final base, drying the sandwich thus formed, and finally stripping off the development support.

5. In color photography a printing process which comprises developing, by differential hardening, a relief image on a colloid layer supported by a sheet of cellophane, combined with transferring the developed image from its cellophane support to another and final base of paper by first soaking the cellophane sheet in water until fully swollen, then mounting it face downwards on the paper base using a dilute solution of gelatine as a mountant, drying the sandwich thus formed and finally stripping off the cellophane support.

In testimony whereof we have signed our names to this specification.

LESLIE WALTER OLIVER.  
WILLIAM GEORGE CLARE. 130